

## UNITED STATES PATENT OFFICE

HANS CAESAR STUHLMANN, OF PREMNITZ, GERMANY, ASSIGNOR TO I. G. FARBNINDUSTRIE AKTIENGESELLSCHAFT, OF FRANKFORT-ON-THE-MAIN, GERMANY

## PROCESS OF TREATING ARTIFICIAL FIBERS

No Drawing. Application filed October 25, 1929, Serial No. 403,547, and in Germany November 16, 1928.

The present invention relates to a process of treating bunches of artificial fibers in a continuous manner in the course of their manufacture and more particularly to an after-treatment of artificial fiber bunches of high total titer on their way from the precipitating bath to the collecting device.

According to my invention bunches of artificial fibers of high total titer and astonishingly good physical properties are obtainable in the viscose spinning process by subjecting the freshly produced fibers collected to form a bunch in the acid moist state, that is, when leaving the precipitating bath, to a tension as high as possible, and by passing them simultaneously through a hot water bath before the usual washing operations and after-treatments take place.

My new operation may be performed in the following manner:

A fiber bunch having a total titer of, for instance, 40,000 to 100,000 deniers is formed by collecting the fibers which are produced by a correspondent plurality of spinning nozzles in a viscose spinning process. The freshly produced and consequently acid-moist fiber bunch is passed through a trough having a length of about 2 to 12 meters, but preferably of 5 meters and being filled with water kept at a temperature of about 70 to 100° C., care being taken that the fiber bunch is completely beneath the surface of the hot water. Simultaneously I stretch the fiber by subjecting them to a high tension of, for instance, 0.5 to 0.8 kilograms per square millimeter. The speed with which the fiber bunch is guided through the bath may vary between 40 to 60 meters per minute. Obviously, the speed is dependent from the length of the water bath. The stretching of the bunches in the water bath may be performed in any known manner, for instance by causing them to run over rods or rolls so that they form an angle on their way or by guiding them over a plurality of rollers of different and adjustable peripheral velocity.

The fiber bunch coming from the precipitating bath is not coagulated throughout. Under the action of the hot liquid hav-

ing a temperature of 70 to 100° C., and under the action of the high tension the fiber bunch soaked with the acid liquid of the precipitating bath is very quickly completely coagulated. The bunch of fibers then is desulfurized, bleached and finished in the usual manner. Thus very valuable products are obtainable. The single fibers of the bunch have for instance a titer of 1.4 deniers and a dry tenacity of about 4 grams and a wet tenacity of about 2 grams, while fibers treated in a hot water bath without tension show a dry tenacity of 2.9 grams and a wet tenacity of 1.2 grams. Furthermore, the material obtained according to my process shows an extremely good luster.

What I claim is:

1. The process which comprises treating in a continuous manner bunches of artificial fibers obtainable by precipitating a viscose solution in an acid precipitating bath in an acid-moist state with hot water, and simultaneously stretching the fibers.

2. The process which comprises collecting artificial fibers made from a viscose solution leaving the precipitating bath to form a bunch of a total titer of about 40,000 to 100,000 deniers, and treating the acid-moist bunch in a water bath of about 70 to 100° C., and simultaneously stretching the fibers.

3. The process which comprises collecting artificial fibers made from a viscose solution leaving the precipitating bath to form a bunch of a total titer of about 40,000 to 100,000 deniers, passing the bunch through a water bath of a length of about 2 to 12 meters being kept at a temperature of about 70 to 100° C., with a drawing speed of about 40 to 60 meters per minute, and subjecting the bunch simultaneously to a tension of about 0.5 to 0.8 kilograms per square meter.

In testimony whereof, I affix my signature.

HANS CAESAR STUHLMANN.

95

100